

# UNITED STATES PATENT OFFICE.

WINFIELD S. POTTER, OF PITTSBURGH, PENNSYLVANIA.

## HEAT TREATMENT AND MANUFACTURE OF WOVEN SCREENS.

1,212,553.

Specification of Letters Patent. Patented Jan. 16, 1917.

No Drawing.

Application filed May 12, 1914. Serial No. 838,029.

*To all whom it may concern:*

Be it known that I, WINFIELD S. POTTER, a citizen of the United States, residing at Pittsburgh, Allegheny county, State of Pennsylvania, have invented certain new and useful Improvements in Heat Treatment and Manufacture of Woven Screens; and I do hereby declare the following to be a full, clear, and exact description of the invention, such as will enable others skilled in the art to which it appertains to make and use the same.

The present invention relates to the manufacture of woven steel screens, that is to say, screens which are formed by the interweaving of crossing bars, rods, or wires, of steel, such as ordinary carbon steel, or manganese steel. The material employed in such manufacture is in the form of rolled bars, coils of rod, or coils of wire, and, in order to facilitate the interweaving, the material is appropriately crimped at the intersection of the bars, rods or wires, in making up the screens. The bars and rods are obtained by rolling from relatively large billets, and the wire is obtained by a similar rolling, succeeded by wire drawing. The bars and rods so rolled and the wire so rolled and wire drawn, contain serious rolling strains and other hardening and stiffening characteristics due to the rolling operation, supplemented, in the case of wire by like effects due to the wire drawing operation.

Inasmuch as carbon steel in a hardened condition is not available for screen making, for the reason that it would not withstand crimping and weaving in that state, it is customary to employ either a very soft steel of low carbon content, or an annealed steel of medium carbon content, and the annealing is frequently effected at a sufficiently high temperature to remove, in part at least the more serious rolling strains, but it is not of a character to remove such segregation of carbids as has occurred in the steel.

The crimping operation is effected either in a press, as, for instance, by making a number of crimps by one motion of the press, or in a continuous manner through crimping rolls of the general character of spur gears, and the bending or crimping is ordinarily done while the bar or rod is cold. In either case, the bar is not embraced or pressed upon at points between the crimps, but is indented and offset on the concave side of each crimp. At these indented and

bended points or sections of the bar, the steel is severely strained. Furthermore, in weaving the bars, the strained sections represent the point of greatest wear and also the point of most severe strain and shock in service. The load of falling materials to be screened, striking heavily upon these high points of the screen, and constantly bumping them during service has the effect of wearing the bar at the crimps, both on their upper and under sides,—on the upper side by the attrition of the materials being screened, and on the other side by rubbing and pounding of the crossing bars. In fact, the wear on the under-side of the bars, at the crimps, is nearly as great as on the upper side, which is perhaps due in part to the fact that, in the screening operation, portions of the gritty materials being screened work their way in between the bars at the crimps. In practice it is found that woven screen bars usually break at the points of intersection of the cross-wires, even when as much as one-half of the original cross-section of the bar remains, so that the screens are more often discarded because a number of their cross-bars are broken than because of the actual wearing through of the bars. In order to obviate these difficulties, and particularly to produce woven screens of high quality from high carbon steel, manganese steel, or the like, I subject the bar, coil of rod, or coil of wire, to a reheating operation at such a temperature as will remove rolling strains, hardness and stiffness, and I prolong the heating operation for a sufficient period to remove segregation, that is to say, to take into solution and fully distribute throughout the steel any carbids that have segregated therein. The effect of this heating operation, however, is to re-crystallize and enlarge the granular structure of the steel, and thereby weaken it. Accordingly, I break down the large crystals and regrain the steel at the same time causing the particles of the regrained steel to firmly cohere. This effect of the combined regraining and increased cohesion, I produce either by immediately crimping the bar or rod while it is still at the temperature to which it has been raised to remove the rolling strains and to restore the carbids into solution; or, if the crimping is to be effected at a subsequent period, I lightly work the rod or bar. In the latter case, the light working will ordinarily be sufficient if the

reduction effected by it is brought about by passing it through two roll passes in each of which the bar is reduced say 2% to 5% in cross section. The bar resulting from this 5 operation will have a fine grain, strong grain cohesion, an absence of segregation, and an absence of the strains, stiffness and hardness referred to. Where the bar or rod is crimped immediately after the heating 10 operation, the working of the steel necessary to break down the enlarged grains and regrain it is effected by the crimping operation itself, the crimping, in such case, being effected in a closed roll pass so that the bar 15 or rod will be worked throughout; or the bar is passed through the crimping rolls and also through a pass at right angles immediately preceding the crimping pass.

After the light reduction above referred 20 to, the bar or rod may be cold-crimped and especially this may be done when the intended screen has large openings and the rod does not have to be sharply crimped. Preferably, however, it is hot-crimped, and 25 if necessary, it is reheated before the hot-crimping, so as to bring it to a suitable temperature to eliminate any possible strains that may have been introduced by the light rolling, and to lessen the strains due to 30 crimping. So also, after the hot-crimping, it may be heat-treated, in a suitable furnace, to relieve whatever strains or other irregularities of condition that may have been introduced during the hot-crimping operation; or, if permitted to cool after hot-crimping, it may be re-heated and then 35 heat-treated at a temperature sufficient to bring the steel to the condition required in the product. A suitable temperature for 40 crimping the rod or bar, without straining, would be, in the case of carbon steels, as low as 500° C.; for manganese steel, it would be preferable to heat the rod or bar, for hot crimping, to a temperature of about 900° C. 45 The heat treatment, after the hot-crimping operation is for the purpose of imparting to the steel a uniform grain structure appropriate to its intimate use. In the case of carbon steel of low carbon content, this 50 may be sufficiently effected by ordinary annealing. In the case of bars of carbon steel having a carbon content higher than that ordinarily employed for screen-making, the hot-crimped bar will have sufficient ductility 55 for weaving if given the heat-treatment ordinarily called "oil tempering and annealing," consisting of heating a bar to above the carbon steel critical range, oil-quenching or otherwise rapidly cooling, heating to 60 say 550° C., or thereabout, and slowly cooling. In the case of manganese steel, the heat-treatment will consist in heating the manganese steel bar or rod to above the critical point ordinarily located at about 65 825° C. to 850° C., and prolonging the heat

at the temperature selected (say 850° C.—900° C.) until the steel is brought to a uniform structure and a fine grain condition followed by rapid cooling, e. g., water-quenching.

In accordance with the foregoing description, it will be noted that the sequence of operations after the preliminary heating and re-rolling may be varied within a considerable range, according to the choice of the 75 operator, which would be determined by the quality of the result which he desires, the kind and analysis of the steel and the particular character of the crimping operation itself. Thus, in some instances, it will be 80 found that the bar or rod may be cold crimped immediately after the light reduction referred to. In other instances, where hot-crimping is practised, the bar or rod may be re-heated either prior to or subsequent to the hot-crimping or both before and after the hot-crimping; and, in still other instances, the final heat-treatment after hot crimping may take place without re-heating, provided that at the termination of 90 the hot-crimping operation the temperature is still sufficiently high to permit of obtaining, either by an appropriate maintenance of the finishing temperature (or any suitable lower temperature), followed by cool- 95 ing steps, the desired condition of the product.

What I claim is:—

1. The method of producing from a rolled steel bar, rod, or wire, a corresponding 100 crimped bar, rod, or wire, for woven screens, which comprises heating the rolled bar, rod, or wire, to such a temperature as to relieve the strains incident to the rolling operation and to bring into solid solution in the metal 105 such carbids as may have segregated therein, working the bar, rod, or wire, sufficiently to condense and refine any coarsely regained portions thereof and ultimately crimping it. 110

2. The method of producing from a rolled steel bar, rod, or wire, a corresponding crimped bar, rod, or wire, for woven screens, which comprises heating the rolled bar, rod, or wire, to such a temperature as to relieve 115 the strains incident to the rolling operation and to bring into solid solution in the metal such carbids as may have segregated therein, working the bar, rod, or wire sufficiently to condense and refine any coarsely regained portions thereof and ultimately 120 crimping it, the working being incidental to the crimping.

3. The method of producing from a rolled steel bar, rod, or wire, a corresponding 125 crimped bar, rod, or wire, for woven screens, which comprises heating the rolled bar, rod, or wire, to such a temperature as to relieve the strains incident to the rolling operation and to bring into solid solution in the metal 130

such constituents as may have segregated therein, working the bar, rod or wire sufficiently to condense and refine any coarsely regrained portions thereof, and ultimately 5 crimping it while still hot, and subsequently heat-treating the metal to bring it to the desired final condition.

4. The method of producing from a rolled steel bar, rod, or wire, a corresponding 10 crimped bar, rod, or wire, for woven screens, which comprises heating the rolled bar, rod, or wire, to such a temperature as to relieve the strains incident to the rolling operation and to bring into solid solution in the metal 15 such constituents as may have segregated therein, working the bar, rod or wire sufficiently to condense and refine any coarsely regrained portions thereof, and ultimately crimping it while still hot, and subsequently 20 heat-treating the metal to bring it to the desired final condition, the heat-treatment being preceded by a reheating operation.

5. The method of producing from a rolled steel bar, rod, or wire, a corresponding 25 crimped bar, rod, or wire, for woven screens, which comprises heating the rolled bar, rod, or wire, to such a temperature as to relieve the strains incident to the rolling operation and to bring into solid solution in the metal

such constituents as may have segregated 30 therein, working the bar, rod, or wire sufficiently to condense and refine any coarsely regrained portions thereof, and ultimately crimping it while still hot, and subsequently 35 heat-treating the metal to bring it to the desired final condition, the hot crimping being preceded by a reheating operation.

6. The method of producing from a rolled steel bar, rod, or wire, a corresponding 40 crimped bar, rod, or wire, for woven screens, which comprises heating the rolled bar, rod, or wire, to such a temperature as to relieve the strains incident to the rolling operation and to bring into solid solution in the metal 45 such constituents as may have segregated 45 therein, working the bar, rod, or wire sufficiently to condense and refine any coarsely regrained portions thereof and ultimately hot-crimping it, subsequently heat-treating the metal to bring it to the desired final 50 condition, and re-heating it both before and after the hot-crimping.

In testimony whereof I affix my signature, in presence of two witnesses.

WINFIELD S. POTTER.

Witnesses:

JOHN C. PENNIE,  
K. R. PENNIE.